

March 1, 1932.

C. E. WETHERALD

1,848,083

METHOD OF FORMING VALVE TAPPETS

Filed Aug. 7, 1929



Fig. 1



Fig. 2



Fig. 3

Inventor  
Charles E. Wetherald  
By Blackworn, Spencer & Flinch-  
attorneys

## UNITED STATES PATENT OFFICE

CHARLES E. WETHERALD, OF FLINT, MICHIGAN, ASSIGNOR TO GENERAL MOTORS CORPORATION, OF DETROIT, MICHIGAN, A CORPORATION OF DELAWARE

## METHOD OF FORMING VALVE TAPPETS

Application filed August 7, 1929. Serial No. 384,067.

This invention relates to valve tappets and more particularly to that type of tappet in which the base or cam-engaging face is formed of one kind of metal, while the stem 5 or shell portion is formed of a different kind of metal.

It has long been recognized that while it is necessary to make the tappet sufficiently large in diameter to provide a proper area of bearing surface between the tappet and the part in which it reciprocates, it is very desirable to keep the weight of the tappets as low and as uniform as possible, in order to increase the engine efficiency and to promote smooth and quiet performance. For this reason, an ideal type of tappet is one in which the upper portion is in the form of a tubular shell and the cam-engaging face is of some suitable material which will withstand the wear caused by the action of the cams against such face.

It has been found that chilled cast iron or certain alloy steels are ideal materials to be employed in the base of such a tappet, since 25 they possess the proper hardness to withstand the constant impact of the cams. It is not necessary or even desirable that the shell portion be formed of the same material as the base, since when chilled cast iron is used 30 it would greatly increase the cost to chill the entire outer surface of the tappet, instead of merely the cam-engaging face. Obviously when alloy steels are employed, the cost would be greatly increased were the entire tappet made of such material. Consequently the practical thing to do is to form 35 the shell of some cheaper material. To cast the shell is not entirely satisfactory since the wall thickness must necessarily be greater and 40 this of course increases the weight which is objectionable. Also, the outside surface of the shell requires considerable machining when cast and if the inside surface is not machined there is a possibility of slightly different weights in the various tappets, due to 45 molding inaccuracies. If the shell be made in the usual manner from solid steel stock, then a large amount of machining is necessary to remove the material in the center.

50 It is therefore an object of this invention to

provide a tappet in which the shell portion is formed of solid stock by the extrusion process. In this process a heated billet of metal is placed in a die and a plunger is forced under considerable pressure into the billet, 55 causing the metal in the latter to flow axially into the space between the plunger and the die, thus forming a tubular shell. At the same time, part of the metal in the billet is forced into engagement with a groove formed 60 in a base member of chilled cast iron, alloy steel or some other suitable material, which has previously been placed in the die. The resulting tappet requires no machining other than a slight grinding operation on its exterior surface to provide a proper bearing surface, and all such tappets are necessarily of exactly the same weight due to the method employed in their manufacture. Such tappets may be produced very rapidly and consequently their cost is comparatively low. 70

Other objects and advantages will be apparent upon referring to the specification and accompanying drawings, in which:

Fig. 1 is a fragmentary sectional view 75 through the center of the dies employed in the manufacture of my improved tappet, showing the base and the heated billet in the die before the act of extrusion has taken place.

Fig. 2 is a view similar to Fig. 1, but showing the position of the parts after the act of extrusion.

Fig. 3 is a fragmentary vertical section 85 through a portion of an internal combustion engine, showing my improved tappet assembled therein.

The reference numeral 10 indicates a stationary die having an aperture 12 therein of the same diameter as that of the tappet to be 90 produced. A movable support 14 fits into the lower end of the aperture 12 and is adapted to be moved up or down by any suitable means. A plunger 16 of the same diameter as that of the inside of the finished tappet 95 is removably mounted in a movable member 18 adapted to be reciprocated by any suitable means which will furnish sufficient pressure to accomplish the act of extrusion to be described later.

The first step in the production of the tappet is to form a base or cam-engaging member 20 of chilled cast iron, alloy steel or other suitable material. An annular groove 22, preferably undercut, is formed in the base. This base is placed in the aperture 12 in such position that the cam engaging face abuts against the support 14, with the groove 22 on the upper side. A billet 24 of any suitable metal, such as ordinary steel, is heated to a temperature sufficiently high to permit the metal to flow when placed under pressure. This heated billet is just enough smaller in diameter than the diameter of the aperture 12 to permit it to be inserted therein, on top of the base 20.

The plunger 16 is then forced under pressure into the billet, and, since the metal cannot flow radially, it must flow axially downward into the groove 22, and upwardly into the space between the plunger 16 and the die 10. Due to the fact that the metal in the billet cannot flow radially, there is no possibility of cracks developing in the outer surface of the metal due to expansion. The thickness of the billet is so proportioned that when the plunger has reached the bottom of its stroke, the metal will have flowed upwardly to such a point as will produce a shell 25 of the desired length. The plunger is then withdrawn, and the tappet is ejected from the die by causing the support 14 to be moved upwardly.

It may not be necessary that the groove 22 be undercut, since when certain combinations of metals are employed, the upper corner of the base tends to expand outwardly during the act of extrusion, and thereby serves to lock the base and shell together. In this case an ordinary straight groove in the base is all that need be provided.

After removal from the die the outside surface of the shell and the cam-engaging face are ground to provide a smooth surface. In Fig. 3 the tappet is shown assembled in an engine 26. The valve operating push rod 28 or valve stem, as the case may be, fits into an aperture 30 drilled through the lower portion of the shell 25 and into the base 20. A passage 32 is formed through the shell to permit the oil which flows down the push rod 28 to drain into the crankcase, thus preventing the tappet from being filled with oil which would increase its weight.

It will thus be seen that I have provided a tappet in which a shell of suitable material is quickly and cheaply formed, and at the same time is interlocked with a base of some material which will provide a proper cam-engaging face. The resulting tappet is very light in weight and yet provides a large amount of bearing area, thus preventing rapid wear. Very little machining is necessary and consequently the tappet may be produced very economically. Obviously

the extrusion process may be employed to form the tappet from a single piece of metal if it is so desired.

It is thought from the foregoing taken in connection with the accompanying drawings that the method of producing this tappet will be readily understood, and that various changes in the method employed may be made without departing from the spirit and scope of the appended claims.

I claim:

1. The method of forming a valve tappet which consists in placing a preformed base in a die, inserting a metal billet in the die adjacent the base, and then forcing a plunger into said billet to simultaneously cause the metal in the billet to flow into interlocking engagement with said base and to flow into the space between the plunger and the die to form the billet into a tubular shell.

2. The method of forming a valve tappet which consists in placing a cam-engaging member having a groove formed therein in a die, inserting a heated metal billet adjacent said member, and then forcing a plunger into said billet to cause the metal in the latter to flow axially into the space between the plunger and the die to form a tubular shell and at the same time to flow axially into the groove to interlock the shell with the cam-engaging member.

3. The method of forming a valve tappet which consists in placing a base having a groove formed therein in a die, inserting a heated metal billet in the die adjacent the base, and then forcing a plunger into the billet thereby extruding the metal into the space between the plunger and the die to form a tubular shell and also into the groove to interlock the base to the shell.

4. The method of forming a valve tappet which consists in placing a cam-engaging member having an undercut annular groove formed therein in a die, inserting a heated metal billet in said die adjacent said member, and then forcing a plunger into said billet to cause the metal in the latter to flow axially into the space between the plunger and the die to form a tubular shell and at the same time to flow axially into the groove to interlock the cam-engaging member with the shell.

In testimony whereof I affix my signature.  
CHARLES E. WETHERALD.

120

125

130